# EUROPEAN PATENT SPECIFICATION

(11) **EP 1 520 911 B1**
(45) Date of publication and mention of the grant of the patent: **09.12.2009**
(21) Application number: 03425647.9
(22) Date of filing: 03.10.2003
(51) Int. Cl.: C14C 9/02, C14C 13/00

(54) **Method for manufacturing leather**
Methode zur Herstellung von Leder
Méthode de fabrication de cuir

(43) Date of publication of application: 06.04.2005
(73) Proprietor: Industria Conciaria Virginia S.p.A., 50050 Ponte a Cappiano - Fucecchio (FI) (IT)
(72) Inventor: Di Palma, Matteo c/o Conceria Virginia S.p.A., 50050 Ponte a Cappiano-Fucecchio Firenze (IT)
(74) Representative: Zambardino, Umberto

(56) References cited:
- EP-A- 0 761 823
- EP-A- 1 087 021
- US-A- 5 658 484

## Description

### Field of Application

In its more general aspect, the present invention relates to the treatment of raw hides for manufacturing leather destined to be used in clothing items, footwear, leather goods.

In particular, the present invention relates to a method for manufacturing a leather having an improved combination of characteristics that make it particularly suitable for the above uses.

### Prior Art

Several methods for manufacturing leather from raw animal hides are known in the art. As a general rule, these methods comprise three manufacturing steps.

In the first manufacturing step, the raw hides undergo a series of treatments having the aim of smoothing and cleaning them so as to make them suitable for being tanned.

The treatments of this first manufacturing step generally include:
- soaking the preserved hides in water in order to recover the umidity lost during their conservation and to remove water-soluble materials such as salts, blood.
- dehairing and liming by treating the hides in suitable dressings with calcium hydroxide and sodium sulphide,
- deliming, i.e. treating the hides with weak acid solutions or salts thereof in order to remove the residual calcium hydroxide,
- treating the hides with enzymatic products (so called "bating") with the aim of removing residual parts (residual hairs and relevant roots) thus smoothing and cleaning the hides and making them suitable for being tanned.

In the second manufacturing step, the cleaned hides are tanned according to any of a variety of conventional methods. Typically the hides are tanned by using a tanning agent of the mineral or vegetal type. In the tanning with a mineral agent, the hides are first treated with a saline and acid solution (so called pickling) and then with a solution of the tanning agent (e.g. chromium sulphate) containing additives facilitating the fixing of the tanning agent to the hide.

Instead, in the tanning with a vegetal agent (typically tannin), the hides are generally first treated with a solution containing tannin and suitable additives and then with an acid solution facilitating the fixing of the tannin to the hide and the removal of the residual tannin.

At this stage the third manufacturing step begins, wherein the tanned hide may undergo a variety of treatments according to the final destination of use and to the desired characteristics to be conferred to the hide itself. For example the hide can be lubricated with a suitable mixture of fats and oils to improve for instance its characteristics of softness, and it can be dyed by using any of the conventional methods known to the skilled in the art.

According to the used dyeing method, also washing characteristics can be conferred to the hides, these characteristics giving the possibility of subjecting the hide to a washing treatment with common household means without incurring in dye release for example on possible fibres coupled with the hide itself.

In some cases, the hides also undergo a retanning treatment for introducing further additives able to confer to the hide additional characteristics, e.g. waterproofing, fulness to the touch, and/or to enhance the previously conferred characteristics.

Although a great deal of methods for treating raw hides for obtaining a leather having one or more characteristics chosen for example among softness, fulness to the touch, waterproofing, washability, elasticity, colour fastness, are thus available to the skilled in the art, it is anyway difficult at present to manufacture a leather having a suitable combination of these characteristics.

In fact, the suitable conferment of these characteristics to the final leather is reached only by accurately controlling a complex series of variables involved by the manufacturing method among which the nature of the additives and solutions used in the various manufacturing steps, pH of the treatment solutions, treatment times.

EP 0761823 discloses a process for the production of household-machine washable and dryable, waterproof, nonflammable, and extremely colorfast leathers from wet blue hides, the process having the advantage that significantly reduced volumes of toxic wastes are generated. The wet blue hides are washed and treated to equalize the pH at the surface and in the interior of the leather and to build at least one wanted end characteristics such as suppleness into the leather. This is followed by the introduction of additional character builders into the pores of the hide and the substitution of one or more softening agents for fats originally present in the pores of the hide. Next there are dyeing and the fixing of previously introduced substances in the pores of the hide. This is followed by refloatation with a hydrophobic waterproofing agent and buffering for pH equalization and increase of the pH. The hides are next treated to impart a pleasing, silky feel to the leather into which the hides are being converted and a hydrophobic silicone which promotes waterproofability and washability; and this is followed by a second fixing step.

EP 1087021 discloses a leather treatment composition (I) comprising: (a) a polysiloxane containing carboxylic acid or carboxylic anhydride groups, where the carboxylic acid groups are in neutralized form; (b) an amphiphilic copolymer prepared from hydrophilic and hydrophobic monomer units; (c) an emulsifier; and (d) an oil or wax. There is also disclosed a leather treatment method involving application of (I) at 1-25 wt. % (based on the leather) from an aqueous liquor of pH 4.0-8.5 during or after retanning, leaving (I) in contact with the leather for 20-150 minutes and adjusting the pH to 3-5, preferably followed by treatment with a 2-4 valent metal salt.

US 5658484 discloses anhydrous and water-containing agents for waterproofing leathers and furs, which comprise a silicone and as emulsifier an alkyl polyalkylol ether carboxylic acid and/or an alkylaryl polyalkylol ether carboxylic acid and/or one of their alkali, alkaline earth, ammonia, amine, or alkanolamine salts. These agents are used for waterproofing, Preferably in retanning or afterwards.

There is thus the need of providing a method for manufacturing leather allowing to confer to the finished product improved characteristics with respect to those conferred by state-of-the-art methods. In particular, there exist the need of providing a washable dyed leather having at the same time good characteristics of softness, fulness to the touch, fastness of the colour, waterproofing and elesticity.

The problem underlying the present invention is that of providing a method for manufacturing leather satisfying all the above needs.

### Summary of the invention

Such a problem is solved, according to the invention, by a method for manufacturing washable leather comprising the preparation, in a conventional way, of tanned hides starting from raw hides and characterised in that it comprises the following additional steps of:
a) subjecting the tanned hides to retanning,
b) subjecting said retanned hides to at least a lubrification treatment with an emulsion obtained by mixing 70-90 parts by weight of an organic phase constituted of synthetic hydrophobic oils and 10-30 parts by weight of a watery phase constituted of an emulsion of silicone compounds.
c) subjecting said retanned and lubricated hides to dyeing with a dyeing agent possibly in association with cationic acrylic resins,
d) subjecting the dyed hides obtained by step c) to a fixing treatment with a watery emulsion comprising silicone compounds and with metallic salts.

According to an embodiment of the invention, the method further comprises, before step b), at least one of the following steps:
- treating said retanned hides with a pH regulating agent so as to enhance the pH to a value of around 6-7,
- treating said retanned hides possibly after having enhanced their pH to 6-7 with a watery solution or watery suspension of acrylic resins.

In the method according to the invention, the preparation of tanned hides starting from raw hides includes the normal operations of cleaning the raw hides so as to get them ready for the tanning and the tanning treatment itself.

The operations of cleaning the raw hides can be carried out in a conventional way by following the above described procedures, which render the hides smooth, clean and hides ready for being tanned.

Preferably, the tanning is carried out by means of a chromium tanning agent so as to obtain hides of the type known as Wet Blue. Such hides can be subjected, before retanning, to a bleaching treatment with sodium hydrosulphite and oxalic acid, the latter as a reducing agent. Such bleaching treatment results being efficient to get rid of superficial dirt and thus it is preferable especially if, in the following manufacturing steps, a light dye is to be given to the hides.

In the method according to the invention, the bleaching treatment is preferably carried out by placing the hides in a conventional apparatus known as tumbler and thus by adding in sequence, the percentages by weight on the weights of the hides to be treated, 100-300% of water, preferably around 200%, 1-3%, preferably 2% by weight of anhydrous sodium hydrosulphate and 0,3-1%, preferably 0,5% of a conventional dislubricating agent chosen among fatty acids and soaps.

The tumbler is then placed in rotation for a period of around 30-90 minutes, preferably 60 minutes and, at the end of the rotation 0,7-1,5% by weight of oxalic acid are added, preferably 1%. After having placed the tumbler again in rotation for around 30-60 minutes, preferably 40 minutes, an abundant washing with running water is then carried out.

In the method according to the invention, the retanning treatment of the hides, possibly having already been subjected to the above described bleaching treatment, is carried out in a conventional way, preferably by using a chromium tanning agent, e.g. powder oxide chromium.

Preferably, the retanning treatment is carried out by adding to the tumbler containing the hides to be treated, in percentages by weight on the weight of the hides, 50-200% of water, preferably around 100%, 5-6% of chromium oxide and 0,5-0,6% of sodium bicarbonate. Then the tumbler is placed in rotation for a period of 2-4 hours, preferably 3 hours and at the end of the rotation an abundant washing with running water is carried out.

In the method according to the invention, the enhancement of the pH of the retanned hides is preferably carried out by adding to the tumbler containing hides, in percentages by weight on the weight of the hides to be treated, 50-200% of water, preferably around 100% and 1,5-3%, preferably 2% of ammonium bicarbonate (pH regulator) so as to enhance the pH to a value of 6-7. Then the tumbler is placed in rotation for a period of 60-120 minutes, preferably 90 minutes and, at the end of the rotation an abundant washing with running water is carried out.

The enhancement of the acid pH typical of the retanned hides to a value around the neutrality advantageously allows to prepare the hides in the best way for the subsequent treating steps and it results to be particularly suitable for obtaining a good softness of the hides in said subsequent steps.

In the method according to the invention, the optional treatment of the retanned hides with the mixture of acrylic resins is preferably carried out in the tumbler containing the hides to be treated by adding therein, in percentages by weight on weight of the hides, 100-300% of water, preferably around 200% and 3-5% of a watery solution of acrylic resins.

Then the tumbler is placed in rotation for a peroiod of 30-90 minutes, preferably 60 minutes and, at the end of the rotation, an abundant washing with running water is carried out.

Preferably, the acrylic resins useful in the method according to the invention are composed of polymers and co-polymers of the methacrylic acid, the percentage by weight of the resins in the solution is of around 40% and the pH of the solution is comprised between 4,2 and 5,5.

The treatment of the retanned hides with the mixture of acrylic resins advantageously confers to the hide the proper degree of fulness to touch.

A very important aspect of the present invention is given by the lubrication step (step b). In accordance with the present invention, such lubrication step is carried out by treating the hides in a tumbler with an emulsion obtained by mixing under agitation 70-90 parts by weight on the total weight of the emulsion of an organic phase constituted of hydrophobic synthetic oils and 10-30 parts by weight of a watery phase constituted of an emulsion of silicone compounds.

The hydrophobic synthetic oils constituting the organic phase preferably have anionic character, i.e. they comprise anionic organic units. A preferred product for the organic phase is sold by Dermacolor s.r.1. with the name of DERMADOL W 300 and it comprises a mixture of syntetical oils able to confer waterproofing to the hide.

The silicone compounds constituting the emulsion of the watery phase are chosen from the group comprising silane and siloxane compounds and respective polymeric products of condensation. A preferred product for the watery phase is constituted of a watery emulsion of dimethylpolysiloxane.

Preferably, the emulsion used in the lubricating process is prepared in situ and it is used in percentages by weight on the weight of the hides to be treated comprised between 8% and 15%. After adding the emulsion to the hides, the tumbler is placed in rotation for a period of 60-120 minutes, preferably 90 minutes and, at the end of the rotation, an abundant washing with running water is carried out.

The above specified lubricating treatment confers to the hides characteristics of softness, waterproofing, transpiration and elasticity desired for the final application.

The lubricated hides as specified above are dryed in a conventional way, e.g. by means of vaccum applications and windy conditioning for then being selected for the following manufacturing steps.

In accordance with a preferred embodiment of the invention, before subjecting the selected hides to dyeing (step c), it is preferred to carry out on the same a second lubricating treatment with the same emulsion used for the first lubrication.

Preferably, for the second lubrication treatment the emulsion is used in proportions from 2% to 8% by weight on the weight of the dryed hides.

This second lubricating treatment allows to improve, i.e. enhancing, the characteristics of softness, waterproofing/transpiration and elasticity already conferred to the hides in the previous lubrication.

In the method according to the invention, the lubricated hides (in one or two steps as specified above) are then subjected to the dyeing treatment.

In accordance with the invention, the dyeing is carried out by adding to the hides to be dyed placed in a tumbler, 100-300% by weight on the weight of the hides of water and 1-6% by weight of a dyeing agent of a conventional type chosen according to the colour which is to be conferred to the final hide. The tumbler is then placed in rotation according to the normal dyeing times.

In accordance with a preferred embodiment of the invention, in the dyeing step, the hides are further treated with a solution containing 1-3% by weight of cationic acrylic resins.

These resins act as auxiliaries for dyeing, facilitating the fixing of the chosen dyeing agent to the hide and thus allow the improvement of the characteristics of fastness of the colour.

The dyeing is generally completed by a fixing step which allows to bind permanently in the pores of the hides all the chemical products used in the previous treatments (es. lubrication and dyeing).

In the method according to the invention, carrying out the fixing by treating the hides in a tumbler with a watery emulsion comprising silicone compounds and with metallic salts has resulted advatageous.

The silicone compounds are preferably chosen from the group comprising silane and siloxane compounds and their respective polymeric products of condensation whereas the nature of the metallic salts varies according to the chosen dyeing agent. Suitable metallic salts are chosen among chromium, aluminium and zirconium salts.

Preferably, the fixing treatment is carried out by adding in the tumbler containing the dyed hides, in percentages by weight on the weight of the hides, 100-300% of water, preferably 200%, 0,5-3% of silicone emulsion and 3-6% of metallic salts.

The leather obtained with the method according to the invention has high qualities and characteristics of softness, waterproofing, transpiration, elesticity, fulness to touch, colour fastnessand stability, washability, fastness to light and to fading, which fully satisfy the standards required by the international rules in this field.

In particular, as regards the characteristic of colour fastness, which is strictly correlated with washability, it has surprisingly been discovered that the leather obtained according to the invention has mean values on the scale of the grey in the range of 4-5 as determined according to the international rule IUF 423.

According to this international rule, samples of dyed leather are coupled with particular non-dyed fabrics, agitated in a neutral solution of synthetic detergent and then rinsed and dryed. At this stage the variations of colour on the samples as well as the degree of migration of the colour on the accompanying fabrics are evaluated by comparing them with the scale of the grey. The results are then expressed in values of the scale of the grey variable from 1 to 5 wherein a significant bleaching of the hide and/or a significant migration of the colour from the hide to the coupling fabric correspond to the minimum value of 1 whereas the maximum value of 5 is given to a leather that, at the end of the test, has no variation of the colour of the leather and/or colouring of the accompanying fabric.

In the case of the leather obtained according to the method of the invention, from washing tests on samples coloured with 50 different colours and associated with accompanying fabrics having fibres of materials chosen among cellulose acetate, cotton, nylon, polyesther, acrilic fibres and wool, mean values have been detected in the range 4-5 both as regards the colour variation of the hide (colour fastness) and the dyeing of the accompanying fabric.

The leather according to the invention also has improved characteristics of transpiration and waterproofing. As regards transpiration, measures on samples of leather carried out on according to the international rule IUP 15 have shown transpiration values (i.e. permeability to water vapour) higher or equal to 10 mg/cm² h and generally comprised between 10 and 15 mg/cm² h.

Instead, as regards waterproofing, measures on samples of leather carried out according to the international rule IUP 10 have shown values of resistance to the penetration of water comprised between 90 and 120 minutes with absorption of water varying from 10% to 15% by weight on the weight of the examined sample of leather.

The leather obtained according to the method of the invention also has excellent elasticity characteristics. In fact, from measures of resistance to the traction (e.g. by means of the rules ISO 3376 or IUP 6) a breaking load higher or equal to 12 N/mm² and a stretch higher or equal to 40% have been detected.

Without being linked to any scientific theory it is believed that the improvement of all these characteristics is reached thanks to the peculiarity of the treatment steps of the hides provided in the method according to the invention and to the peculiarity of the chemical compositions used in these treatment steps.

More particularly, it is believed that the improved characterstics of colour fastness, washability, fastness to light and to fading (characteristics strictly connected one another) are reached thanks to the use, during the dyeing steps, of dyeing agents selected together in association with cationic acrylic resins as auxiliaries of dyeing and of the peculiarity of the fixing of said agents to the hide.

In particular, the use of the above dyeing agents together with the auxiliaries of dyeing in the above described ways would allow the dyes themselves to adequately penetrate into the pores of the hides whereas by means of the fixing said dyes would form very strong chemical bonds with the hides in correspondence with active sites in their pores.

Instead, as regards the improvement of the characteristics of softness, waterproofing, transpiration and elesticity it is believed that such improvement is reached thanks to the use of the particular emulsions with their oily and watery phases used in the lubricating steps.

In particular, the use of these particular emulsions in the above indicated proportions and modes would allow a sufficient and uniform penetration of the hide by the fatty substances contained in the emulsions, which fatty substances would thus form interactions of various type with the collagene matrix of the hide. The bond among fatty substances of the hide would be then highly reinforced during the fixing treatment thus ensuring to the hide the desired characteristics of softness, transpiration, waterproofing and elesticity.

The main advantage of the leather obtained through the method according to the invention lies in the fact that it can be efficiently subjected to washing with neutral detergent at a temperature of around 40°C without any substantial structural alteration of the hide (e.g. loss of elasticity and/or shrinking) and of the softness, and without any release and variation of colour.

Therefore, the leather obtained according to the invention is advantageously suitable for being used as it is alone or coupled to other natural or synthetic fibres for manufacturing washable items, e.g in the field of clothing, footwear, leather goods and furnishing.

In this use, advantageously the leather does not need further specific finishing treatments.

The method according to the invention is efficiently appliable to all the raw hides of natural origin with particular reference to bovine and ovogoaty hides.

## Claims

1. A method for manufacturing washable leather comprising the preparation, in a conventional way, of tanned hides starting from raw hides and **characterised in** the fact that it comprises the additional steps of:
a) subjecting the tanned hides to retanning,
b) subjecting said retanned hides to at least a lubricating treatment with an emulsion obtained by mixing 70-90 parts by weight of an organic phase constituted of synthetic hydrophobic oils and 10-30 parts by weight of a watery phase constituted of an emulsion of silicone compounds,
c) subjecting said retanned and lubricated hides to dyeing with a dyeing agent possibly in association with cationic acrylic resins,
d) subjecting the dyed hides obtained from step c) to a fixing treatment with a watery emulsion comprising silicone compounds and metallic salts.

2. A method according to claim 1, further comprising before step b), at least one of the following steps:
- treating said retanned hides with a pH regulating agent so as to enhance the pH to a value of around 6-7,
- treating said retanned hides possibly after having enhanced their pH to 6-7 with a watery solution of acrylic resins.

3. A method according to claim 1 or claim 2, wherein said retanning step is carried out by treating the tanned hides in a watery bath comprising the following ingredients in percentages by weight on the weight of the hides:
50-200% water,
5-6% cromium oxide
0,5-0,6% sodium bicarbonate.

4. A method according to any of the previous claims, wherein two lubricating steps of said retanned hides are provided by means of a treatment of the same respectively with 8-15% and 2-8% by weight on the weight of the hides of said emulsion obtained by mixing 70-90 parts by weight of an organic phase constituted of synthetic hydrophobic oils and 10-30 parts by weight of a watery phase constituted of an emulsion of silicone compounds.

5. A method according to claim 4, wherein said synthetic oils comprise anionic organic units.

6. A method according to claim 4 or claim 5, wherein said silicone compounds are chosen from the group comprising silane and siloxane compounds and respective polymeric products of condensation.

7. A method according to any of the claims from 4 to 6, wherein said watery phase is constituted of an emulsion of dimethylpolysiloxane.

8. A method according to any of the previous claims, wherein said dyeing step is carried out by treating said retanned and lubricated hides in a watery bath comprising the following ingredients in percentages by weight on the weight of the hides:
100-300% water
1-6% dyeing agent
1-3% cationic acrylic resins.

9. A method according to any of the previous claims, wherein said fixing step is carried out by treating the dyed hides in a watery bath comprising the following ingredients in percentages by weight on the weight of the hides:
100-300% water
0,5-3% emulsion comprising silicone compounds
3-6% metallic salts.

10. A method according to any of the claims 2 to 9, wherein said treating step of the hides retanned with a pH regulating agent is carried out in a watery bath comprising the following ingredients in percentages by weight on the weight of the hides:
50-200% water,
1,5-3% ammonium bicarbonate.

11. A method according to any of the claims 2 to 10, wherein said treating step of the hides retanned with a watery solution of acrylic resins is carried out in a watery bath comprising the following ingredients in peercentages by weight on the weight of the hides:
100-300 % water,
3-5% watery solution of acrylic resins.

12. A method according to any of the previous claims, wherein the conventional preparation of the tanned hides provides the use of a chromium tanning agent so as to obtain Wet Blue hides.

13. A method according to any of the previous claims, further comprising before the retanning step (step a), the step of subjecting the tanned hides to a bleaching treatment with sodium hydrosulphite and oxalic acid.

14. A method according to claim 13, wherein said bleaching treatment of the retanned hides is carried out in a watery bath comprising the following ingredients in percentages by weight on the weight of the hides:
100-300% water
1-3% sodium hydrosulphite
0,3-1% dislubricating agent chosen among fatty acids and soaps.
0,7-1,5% oxalic acid.

15. Use of a washable leather obtained by the method according to any of the claims 1 to 14 in the manufacturing of clothing items, footwear, leather goods and furnishing.

16. Chemical composition for use in the lubricating treatment of retanned hides consisting of 70-90% by weight on the weight of the composition of an organic phase constituted of synthetic hydrophobic oils and 10-30% by weight on the weight of the composition of a watery phase constituted of an emulsion of silicone compounds, said organic and watery phases being mixed one another before said use in order to form an emulsion.

## Patentansprüche

1. Verfahren zum Herstellen eines waschbaren Leders umfassend die Herstellung, in einer üblicherweise, gegerbter Häute ausgehend von rohen Häuten und **dadurch gekennzeichnet, dass** es die zusätzlichen Schritte umfasst:
a) Unterwerfen der gegerbten Häute einem erneuten Gerben,
b) Unterwerfen der erneut gegerbten Häute mindestens einer einfettenden Behandlung mit einer Emulsion erhältlich durch Mischen 70-90 Gewichtsteile einer organischen Phase bestehend aus synthetischen hydrophoben Ölen und 10-30 Gewichtsteilen einer wässrigen Phase bestehend aus einer Emulsion von Silikonverbindungen,
c) Unterwerfen der erneut gegerbten und eingefetteten Häute einem Färben mit einem Färbemittel, gegebenenfalls in Verbindung mit kationischen Acrylharzen,
d) Unterwerfen der gefärbten Häute aus Schritt c) einer Fixierungsbehandlung mit einer wässrigen Emulsion umfassend Silikonverbindungen und metallische Salze.

2. Verfahren nach Anspruch 1, ferner umfassend vor Schritt b) mindestens einen der folgenden Schritte:
- Behandlung der erneut gegerbten Häute mit einem pH einstellenden Mittel, um den pH auf einen Wert um 6-7 zu verbessern,
- Behandeln der erneut gegerbten Häute, gegebenenfalls nach der Verbesserung ihres pH's auf 6-7 mit einer wässrigen Lösung von Acrylharzen.

3. Verfahren nach Anspruch 1 und 2, in dem der Schritt des erneuten Gerbens durchgeführt wird durch Behandlung der gegerbten Häute in einem wässrigen Bad umfassend die folgenden Zutaten in Gewichtsprozenten basierend auf dem Gewicht der Häute:
- 50-200% Wasser,
- 5-6% Chromoxid,
- 0,5-0,6% Natriumbicarbonat.

4. Verfahren nach irgendeinem der vorhergehenden Ansprüche, in dem zwei Einfettungsschritte der erneut gegerbten Häute durchgeführt werden mittels einer Behandlung derselben entsprechend mit 8-15% und 2-8% Gewichtprozenten basierend auf dem Gewicht der Häute einer Emulsion erhalten durch Mischen von 70-90 Gewichtsteilen einer organischen Phase bestehenden aus synthetischen hydrophoben Ölen und 10-30 Gewichtsteilen einer wässrigen Phasen bestehend aus einer Emulsion von Silikonverbindungen.

5. Verfahren nach Anspruch 4, in dem die synthetischen Öle anionische organische Einheiten umfassen.

6. Verfahren nach Anspruch 4 oder 5, indem die Silikonverbindungen ausgewählt werden aus der Gruppe umfassend Silan- und Siloxan-Verbindungen und entsprechende polymere Kondensationsprodukte.

7. Verfahren nach irgendeinem der Ansprüche 4 bis 6, in dem die wässrige Phase aus einer Emulsion von Dimethylpolysiloxan besteht.

8. Verfahren nach irgendeinem der vorhergehenden Ansprüche, in dem der Färbeschritt durchgeführt wird durch Behandlung der erneut gegerbten und eingefetteten Häute in einem wässrigen Bad umfassend die folgenden Zutaten in Gewichtsprozenten basierend auf dem Gewicht der Häute:
- 100-300% Wasser,
- 1-6% Färbemittel,
- 1-3% kationische Acrylharze.

9. Verfahren nach irgendeinem der vorhergehenden Ansprüche, in dem der Fixierungsschritt durchgeführt wird durch Behandlung der gefärbten Häute in einem wässrigen Bad umfassend die folgenden Zutaten in Gewichtsprozenten basierend auf dem Gewicht der Häute:
- 100-300% Wasser,
- 0,5-3% einer Emulsion umfassend Silikonverbindungen,
- 3-6% metallische Salze.

10. Verfahren nach irgendeinem der Ansprüche 2 bis 9, in dem der Behandlungsschritt der erneut gegerbten Häute mit einem pH einstellenden Mittel durchgeführt wird in einem wässrigen Bad umfassend die folgenden Zutaten in Gewichtsprozenten basierend auf dem Gewicht der Häute:
- 50-200% Wasser,
- 1,5-3% Ammoniumbicarbonat.

11. Verfahren nach irgendeinem der Ansprüche 2 bis 10, in dem der Behandlungsschritt der erneut gegerbten Häute mit einer wässrigen Lösung von Acrylharzen durchgeführt wird in einem wässrigen Bad umfassend die folgenden Zutaten in Gewichtsprozenten basierend auf dem Gewicht der Häute:
- 100-300% Wasser,
- 3-5% einer wässrigen Lösung von Acrylharzen.

12. Verfahren nach irgendeinem der vorhergehenden Ansprüche, in dem die übliche Behandlung der gegerbten Häute die Verwendung eines Chromgerbemittels umfasst, um somit Wet Blue Häute zu erhalten.

13. Verfahren nach irgendeinem der vorhergehenden Ansprüche, ferner umfassend vor dem Schritt der erneuten Gerbung (Schritt a) den Schritt des Aussetzens der gegerbten Häute einer Bleichbehandlung mit Natriumhydrosulphit und Oxalsäure.

14. Verfahren nach Anspruch 13, in dem die Bleichbehandlung der erneut gegerbten Häute durchgeführt wird in einem wässrigen Bad umfassend die folgenden Zutaten in Gewichtsprozenten basierend auf dem Gewicht der Häute:
- 100-300% Wasser,
- 1-3% Natriumhydrosulphit,
- 0,3-1% entfettendes Mittel ausgewählt aus Fettsäuren und Seifen,
- 0,7-1,5% Oxalsäure.

15. Verwendung eines waschbaren Leders erhalten nach einem Verfahren nach irgendeinem der Ansprüche 1 bis 14 in der Herstellung von Bekleidungsstücken, Schuhwerk, Lederwaren und Möbel.

16. Chemische Zusammensetzung zur Verwendung in der einfettenden Behandlung von erneut gegerbten Häuten bestehend aus 70-90 Gewichtsprozenten basierend auf dem Gewicht der Zusammensetzung einer organischen Phase bestehend aus synthetischen hydrophoben Ölen und 10-30 Gewichtsprozenten basierend auf der Zusammensetzung einer wässrigen Phase bestehend aus einer Emulsion von Silikonverbindungen, wobei die organischen und wässrigen Phasen miteinander vermischt werden, um eine Emulsion auszubilden.

## Revendications

1. Procédé de fabrication d'un cuir lavable comprenant la préparation, de manière conventionnelle, de cuirs tannés à partir de cuirs bruts et **caractérisé** dans le fait qu'il comprend les étapes supplémentaires consistant à :
a) soumettre les cuirs tannés à un retannage,
b) soumettre lesdits cuirs retannés à au moins un traitement lubrifiant avec une émulsion obtenue en mélangeant 70 à 90 parties en poids d'une phase organique constituée d'huiles hydrophobes synthétiques et 10 à 30 parties en poids d'une phase aqueuse constituée d'une émulsion de composés de silicone,
c) soumettre lesdits cuirs retannés et lubrifiés à une teinture avec un agent de teinture, éventuellement en association avec des résines acryliques cationiques,
d) soumettre les cuirs teints obtenus à partir de l'étape c) à un traitement fixateur avec une émulsion aqueuse comprenant des composés de silicone et des sels métalliques.

2. Procédé selon la revendication 1, comprenant en outre avant l'étape b), au moins une des étapes suivantes :
- traitement desdits cuirs retannés avec un agent régulateur de pH de façon à porter le pH à une valeur autour de 6-7,
- traitement desdits cuirs retannés éventuellement après avoir porté leur pH à 6-7 avec une solution aqueuse de résines acryliques.

3. Procédé selon la revendication 1 ou la revendication 2, dans lequel ladite étape de retannage est effectuée en traitant les cuirs tannés dans un bain aqueux comprenant les ingrédients suivants en pourcentages en poids sur le poids des cuirs :
50 à 200% d'eau,
5 à 6% d'oxyde de chrome,
0,5 à 0,6% de bicarbonate de sodium ;

4. Procédé selon l'une quelconque des revendications précédentes, dans lequel deux étapes de lubrification desdits cuirs retannés sont prévues au moyen d'un traitement de ces derniers avec respectivement 8 à 15% et 2 à 8% en poids sur le poids des cuirs de ladite émulsion obtenue en mélangeant 70 à 90 parties en poids d'une phase organique constituée d'huiles hydrophobes synthétiques et 10 à 30 parties en poids d'une phase aqueuse constituée d'une émulsion de composés de silicone.

5. Procédé selon la revendication 4, dans lequel lesdites huiles synthétiques comprennent des unités organiques anioniques.

6. Procédé selon la revendication 4 ou la revendication 5, dans lequel lesdits composés de silicone sont choisis dans le groupe comprenant des composés de silane et de siloxane et des produits polymériques respectifs de condensation.

7. Procédé selon l'une quelconque des revendications 4 à 6, dans lequel ladite phase aqueuse est constituée d'une émulsion de diméthylpolysiloxane.

8. Procédé selon l'une quelconque des revendications précédentes, dans lequel ladite étape de teinture est effectuée en traitant lesdits cuirs retannés et lubrifiés dans un bain aqueux comprenant les ingrédients suivants en pourcentages en poids sur le poids des cuirs :
100 à 300% d'eau,
1 à 6% d'agent de teinture,
1 à 3% de résines acryliques cationiques.

9. Procédé selon l'une quelconque des revendications précédentes, dans lequel ladite étape de fixation est effectuée en traitant les cuirs teints dans un bain aqueux comprenant les ingrédients suivants en pourcentage en poids sur le poids des cuirs :
100 à 300% d'eau,
0,5 à 3% d'émulsion comprenant des composés de silicone,
3 à 6% de sels métalliques.

10. Procédé selon l'une quelconque des revendications 2 à 9, dans lequel ladite étape de traitement des cuirs retannés avec un agent régulateur de pH est effectuée dans un bain aqueux comprenant les ingrédients suivants en pourcentage en poids sur le poids des cuirs :
50 à 200% d'eau,
1,5 à 3% de bicarbonate d'ammonium.

11. Procédé selon l'une quelconque des revendications 2 à 10, dans lequel ladite étape de traitement des cuirs retannés avec une solution aqueuse de résines acryliques est effectuée dans un bain aqueux comprenant les ingrédients suivants en pourcentage en poids sur le poids des cuirs :
100 à 300% d'eau,
3 à 5% de solution aqueuse de résines acryliques.

12. Procédé selon l'une quelconque des revendications précédentes, dans lequel la préparation conventionnelle des cuirs tannés prévoit l'utilisation d'un agent de tannage au chrome de façon à obtenir des cuirs en bleu humide.

13. Procédé selon l'une quelconque des revendications précédentes, comprenant en outre avant l'étape de retannage (étape a), l'étape consistant à soumettre les cuirs tannés à un traitement de blanchiment avec de l'hydrosulfite de sodium et de l'acide oxalique.

14. Procédé selon la revendication 13, dans lequel ledit traitement de blanchiment des cuirs tannés est effectué dans un bain aqueux comprenant les ingrédients suivants en pourcentages en poids sur le poids des cuirs :
100 à 300% d'eau,
1 à 3% d'hydrosulfite de sodium,
0,3 à 1% d'agent délubrifiant choisi parmi les acides gras et les savons
0,7 à 1,5% d'acide oxalique.

15. Utilisation d'un cuir lavable obtenu par le procédé selon l'une quelconque des revendications 1 à 14 dans la fabrication de vêtements, de chaussures, d'articles de maroquinerie et d'ameublements.

16. Composition chimique destinée à être utilisée dans le traitement de lubrification des cuirs retannés composée de 70 à 90% en poids sur le poids de la composition d'une phase organique constituée d'huiles hydrophobes synthétiques et de 10 à 30% en poids sur le poids de la composition d'une phase aqueuse constituée d'une émulsion de composés de silicone, lesdites phases organique et aqueuse étant mélangées l'une avec l'autre avant ladite utilisation afin de former une émulsion.
